# EUROPEAN PATENT SPECIFICATION

(11) **EP 4 382 662 B1**
(45) Date of publication and mention of the grant of the patent: **23.04.2025**
(21) Application number: 22211462.1
(22) Date of filing: 05.12.2022
(51) Int. Cl.: D21F 9/00, D21F 11/04

(54) **METHOD FOR PRODUCTION OF A MULTI-PLY PAPERBOARD**
VERFAHREN ZUR HERSTELLUNG EINER MEHRLAGIGEN PAPPE
PROCÉDÉ DE FABRICATION D'UN CARTON MULTICOUCHE

(43) Date of publication of application: 12.06.2024
(73) Proprietor: Billerud Aktiebolag (publ), 169 27 Solna (SE)
(72) Inventor: ATTEMALM, Adam, 653 50 Karlstad (SE); HAGELQVIST, Magnus, 656 38 Karlstad (SE)
(74) Representative: Kransell & Wennborg KB

(56) References cited:
- EP-A1- 0 511 186
- DE-A1- 102010 029 617
- SE-A1- 1 751 582
- US-A- 5 560 808
- US-A1- 2019 211 503

## Description

### TECHNICAL FIELD

The present disclosure relates to the field of multi-ply paperboards.

### BACKGROUND

Paperboards are commonly made of one ply or out of two or more plies, wherein the latter is referred to as multi-ply paperboards. Multi-ply paperboards are used in for example packaging, such as in liquid packaging board (LPB).

When a multi-ply paperboard is provided, it is important to prevent that cracks are formed to maintain appearance. Moreover, when the multi-ply paperboard is used in packaging, it is important to hinder contamination of the product contained in the package. A method for making a multi-ply paperboard is for example known from SE 1 751 582 A1.

### SUMMARY

Multi-ply paperboards, namely paperboards having two or more plies, are commonly used in packaging. In all boards used in packaging, and especially for LPB, it is important that the board do not crack upon folding it into a package.

Accordingly, the present disclosure provides the following listing of itemized embodiments:
1. A method for making a multi-ply paperboard, wherein the method comprises the following steps:
   a) forming a first web from a first furnish comprising fibres on a first forming wire wherein the first furnish is applied on the first forming wire using a first jet speed at a first jet-to-wire speed difference, wherein the first jet-to-wire speed difference is in the range of: +15 to +30 m/min, such as +16 to +25 m/min or -15 to -30 m/min, such as -16 to -25 m/min;
   b) forming a second web from a second furnish comprising fibres on a second forming wire using a second jet speed, wherein the second jet speed is closer to the speed of the second forming wire than the first jet speed to the speed of the first forming wire;
   c) forming a third web from a third furnish comprising fibres on a third forming wire using a third jet speed, wherein the third jet speed is closer to the speed of the third forming wire than the first jet speed to the speed of the first forming wire;
   d) causing the second web to oscillate in a direction transverse to the machine direction (MD), wherein the stroke length in the oscillation of the second web is 10-35 mm; and
   e) combining the first, second and third webs into the multi-ply paperboard, wherein the first web forms a top-ply, the second web forms a middle ply and the third web forms a back-ply in the multi-ply paperboard.
2. The method of item 1, wherein in step d) further comprising causing the third web to oscillate in a direction transverse to the machine direction.
3. The method of item 1 or 2, wherein the first jet-to-wire speed ratio is above 1.
4. The method of item any one of the preceding items, wherein the first jet-to-wire speed ratio is 1.007 -1.05, such as 1.008-1.04.
5. The method of any one of the preceding items, wherein the second jet-to-wire speed ratio is 1.007-1.03, such as 1.008-1.02.
6. The method of any one of the preceding items, wherein the oscillation(s) in step d) is/are carried out by (a) breast roll shaker(s).
7. The method of any one of the preceding items, wherein the stroke length in the oscillation in step d) of the second web is 12-30 mm, such as 15-30 mm.
8. The method of any one of the items 2-8, wherein the stroke length in the oscillation in step d) of the third web is 8-25 mm, such as, 10-23 mm.
9. The method of any one of the preceding items, wherein the third jet-to-wire speed ratio is above 1, such as 1.007-1.02.
10. The method of any one of the preceding items, wherein the wire speed of all forming wires is 400-1000 m/min, such as 500-900 m/min.
11. The method of any one of the preceding items, wherein the second furnish comprises mechanical pulp, such as chemi-thermomechanical pulp (CTMP).
12. The method of any one of the preceding items, wherein the second furnish comprises broke pulp.
13. The method of any one of the preceding items, wherein the fibres of the third furnish are unbleached.
14. The method of any one of the preceding items, wherein the fibres of the first furnish are bleached.
15. The method of any one of the preceding items, wherein the fibres of the second furnish are unbleached.
16. The method of any one of the preceding items, wherein a MD/cross-direction (CD)-tensile strength ratio is above or equal to 1.7, such as above or equal to 2, such as 2-3.3 in the top ply, wherein the tensile strength is measured according to ISO 1924-3:2011.
17. The method of any one of the preceding items, wherein the MD/CD-tensile strength ratio is above or equal to 1.1, such as 1.1-1.5 in the back ply, wherein the tensile strength is measured according to ISO 1924-3:2011.
18. The method of any one of the preceding items, wherein the MD/CD-tensile strength ratio is above or equal to 1.3, such as 1.3-1.9 in the middle ply, wherein the tensile strength is measured according to ISO 1924-3:2011.
19. The method of any one of the preceding items, wherein the MD/CD-tensile strength ratio is 1.6-2.0 for the whole board, wherein the tensile strength is measured according to ISO 1924-3:2011.
20. The method of any one of the preceding items, wherein the MD/CD tensile strength ratio is higher for the top ply than for the back ply.
21. The method of any one of the preceding items, wherein the MD/CD tensile strength ratio is higher for the middle ply than for the back ply.
22. The method of any one of the preceding items, wherein the second furnish is applied on the second forming wire at a second jet-to-wire speed difference, which is in the range of:
   +4 to +14 m/min, such as +6 to +11 m/min, or
   -4 to -14 m/min, such as -6 to -11 m/min.
23. The method of any one of the preceding items, wherein the third furnish is applied on the third forming wire at a third jet-to-wire speed difference of:
   +4 to +14 m/min, such as +6 to +11 m/min, or
   -4 to -14 m/min, such as -6 to -11 m/min.
24. The method of any one of any one of the preceding items, wherein the third jet speed is closer to the speed of the third forming wire than the second jet speed to the speed of the second forming wire.
25. The method of any one of the preceding items, wherein the grammage according to ISO 536:2019 of the paperboard is 100-450 g/m², such as 120-350 g/m², such as 125-300 g/m².
26. The method of any one of the preceding items, wherein the grammage according to ISO 536:2019 of the top ply is 40-100 g/m².
27. The method of any one of preceding items, wherein the grammage according to ISO 536:2019 of the middle ply is 75-175 g/m².
28. The method of any one of preceding items, wherein the grammage according to ISO 536:2019 of the back-ply ply is 25-175 g/m², such as 25-75 g/m², such as 75-175 g/m².
29. The method of any one of the preceding items, wherein the multi-ply paperboard is coated on the top-ply.
30. The method of any one of the preceding items, wherein the frequency in the oscillation in step d) is 130-650 rpm, such as 250-580 rpm, for the oscillated web(s).
31. The method of any one of the preceding items, wherein the specific formation according to SCAN-P 92:09 for the middle ply is 0.60-0.90 √g/m, such as 0.65-0.85 √g/m.
32. The method of any one of the preceding items, wherein the specific formation according to SCAN-P 92:09 for the back ply is 0.60-0.90 √g/m, such as 0.65-0.85 √g/m.
33. The method of any one of the preceding items, wherein the specific formation according to SCAN-P 92:09 for the whole board is 0.60-0.80 √g/m, such as 0.70-0.80 √g/m.
34. A method for making a two-ply paperboard, wherein the method comprises the following steps:
   i. forming a top ply web from a top ply furnish comprising fibres on a top ply forming wire wherein the top ply furnish is applied on the top ply forming wire using a first jet speed at a first jet-to-wire speed difference, wherein the first jet-to-wire speed difference is in the range of:
      +12 to +30 m/min, such as +14 to +25 m/min or
      -12 to -30 m/min, such as -14 to -25 m/min
   ii. forming a back ply web from a back ply furnish comprising fibres on a back ply forming wire using a second speed, wherein the second jet speed is closer to the second forming wire speed than the first jet speed to the first forming wire speed;
   iii. causing the back ply web to oscillate in a direction transverse to the MD, wherein the stroke length in the oscillation of the back ply web is 10-35 mm; and
   iv. combining the top ply web and back ply webs into the two-ply paperboard, wherein the top-ply web forms a top-ply and the back-ply web forms a back-ply in the two-ply paperboard.

The inventors have realized that the above methods reduce the cracking tendency by producing a board having a top ply in which the tensile strength is about 2-3 times higher in the machine direction (MD) than in the cross direction (CD) and by the formation of a middle ply, in case of at least three plies in the board, and the formation of the back ply, in case of a two-ply board, in which the variations in local grammages is minimised.

### DETAILED DESCRIPTION

As a first aspect of the present disclosure, there is provided a method for making a multi-ply paperboard, wherein the method comprises the following steps:
a) forming a first web from a first furnish comprising fibres on a first forming wire wherein the first furnish is applied on the first forming wire using a first jet speed at a first jet-to-wire speed difference, wherein the first jet-to-wire speed difference is in the range of:
   +15 to +30 m/min, such as +16 to +25 m/min or
   -15 to -30 m/min, such as -16 to -25 m/min;
b) forming a second web from a second furnish comprising fibres on a second forming wire using a second jet speed, wherein the second jet speed is closer to the speed of the second forming wire than the first jet speed to the speed of the first forming wire;
c) forming a third web from a third furnish comprising fibres on a third forming wire using a third jet speed, wherein the third jet speed is closer to the speed of the third forming wire than the first jet speed to the speed of the first forming wire;
d) causing the second web to oscillate in a direction transverse to the machine direction (MD), wherein the stroke length in the oscillation of the second web is 10-35 mm;
e) combining the first, second and third webs into the multi-ply paperboard, wherein the first web forms a top-ply, the second web forms a middle ply and the third web forms a back-ply in the multi-ply paperboard.

By using a jet-to-wire-speed difference in formation of the top ply being greater than the jet-to-wire-speed difference in formation of the middle ply and back ply, the fibres in the top ply will be more oriented in the MD than the fibres in the middle ply and back ply.

As an example, the jet-to-wire speed difference is +20 m/min if the jet speed is 720 m/min and the wire speed is 700 m/min and -20 m/min if the jet speed is 700 m/min and the wire speed is 720 m/min. In each case, the jet-to-wire-speed difference is greater than when the jet speed is 710 m/min and the wire speed is 700 m/min or when the jet speed is 700 m/min and the wire speed is 710 m/min.

The combination of using a jet-to-wire speed difference in the range of +15 to +30 m/min or -15 to -30 m/min in the formation of the first web and oscillation at certain stroke length of the second web has been found to produce a multi-ply paperboard with minimized crack formation upon folding.

When the second web is oscillated with a stroke length in the range of 10-35 mm, the fibres in the second web are caused to be more oriented with the cross direction (CD), i.e. the direction transverse to the machine direction. Moreover, local accumulations of flocs of fibres are evened out. As a consequence, the formation is improved. The inventors have discovered that the tensile strength ratio in MD/CD obtained by the jet-to-wire speed difference for the top ply in combination with the obtained formation of the middle ply is beneficial in reduction of cracks when the paperboard is folded.

For these effects, it is not decisive if the jet is faster than the wire, i.e. a positive speed difference, or slower than the wire, i.e. a negative speed difference. The fibre-orienting effect will be obtained in either case. Nevertheless, it is preferred that the speed difference is positive since a lower fibre concentration in the headbox can be used, which is beneficial since it leads to a better formation of the plies.

Typically, the second and third webs are oscillated in the CD. Thereby, the formation is improved both in the middle ply and the back ply, which is even further beneficial for reduction of cracks when the paperboard is folded.

Typically, the second furnish is applied on the second forming wire at a second jet-to-wire speed difference in the range of:
+4 to +14 m/min, such as +6 to +11 m/min, or
-4 to -14 m/min, such as -6 to -11 m/min.

The third furnish is, typically, applied on the third forming wire at a third jet-to-wire speed difference of, which is in the range of:
+4 to +14 m/min, such as +6 to +11 m/min, or
-4 to -14 m/min, such as -6 to -11 m/min.

In theory the speed difference should be just above, or below, 0, such as ±1 or ±2 m/min to provide good formation. However, due to limitations in equipment it is challenging to maintain such small difference. At a speed difference close to 0 there is a risk that the speed difference at some point will be 0 due to limitations in the equipment and at such point the formation is impaired. The inventors have now realized that by conducting an oscillations step, the jet-to-wire speed difference can instead be not less than ±4 m/min. Such a speed difference together with oscillation provides a more robust system as well as satisfactory sheet formation. By more robust is meant that risk that the speed difference at some point will be 0 is avoided or at least minimized.

Moreover, the jet-to-wire speed difference is typically not more than ±14 m/min as the formation is not improved above such a speed difference. The third jet speed is, typically, closer to the speed of the third forming wire than the second jet speed to the speed of the second forming wire. Thereby the difference in speed in the formation of the second fibre web is greater than the difference in speed in the formation of the third fibre web.

Formation is a measure of how even the surface is, i.e. that there are as few fibre flocs as possible and that the fibres are evenly distributed in all directions. A low formation is beneficial for crack resistance. Formation is measured according to SCAN-P 92:09. For the middle ply the formation is preferably 0.60-0.90 √g/m, such as 0.65-0.85 √g/m. For the back ply the formation is preferably 0.60-0.90 √g/m, such as 0.65-0.85 √g/m.

Typically, the wire speed of all forming wires is 400-1000 m/min, such as 500-900 m/min. The speed of all forming wires are, typically, the same.

The jet-to-wire speed ratio is the jet speed divided by the wire speed. By using the jet-to-wire speed difference in combination with wire speed, the jet-to-wire speed ratio can be calculated. As it is preferred the speed difference is positive, it is consequently preferred that first jet-to-wire speed ratio is above 1. Typically, the first jet-to-wire speed ratio is 1.007 -1.050, such as 1.008-1.040. Typically, the second jet-to-wire speed ratio is 1.007-1.030, such as 1.008-1.020. Typically, the third jet-to-wire speed ratio is above 1, such as 1.007-1.020.

The oscillation(s) in step d) is/are, typically, carried out by (a) breast roll shaker(s). A breast roll shaker shakes the breast roll cross-directionally and breaks up fibre flocs by creating shear forces on the web. Breast roll(s) are typically located downstream and directly after the headbox in the forming section of a paper machine. A breast roll shaker shakes the breast roll.

Preferably, the stroke length in the oscillation in step d) of the second web is 12-30 mm, such as 15-30 mm. Typically, if the third web is oscillated the stroke length in the oscillation in step d) of the third web is 8-25 mm, such as, 10-23 mm. Typically, the frequency in the oscillation in step d) is 130-650 rpm, such as 250-580 rpm, for the oscillated web(s). That is, the second web is oscillated with such frequency as well as the third web, if oscillated. The inventors have realized that the stroke length has a bigger impact on the formation of the web than the frequency.

MD/CD-tensile strength ratio is an indication of the extent to which the fibres are oriented in the MD (a higher ratio corresponds to more MD-oriented fibres). In the top-ply the MD/CD tensile strength ratio is typically above or equal to 1.7, such as above or equal to 2, such as 2-3.3. In the back ply, the MD/CD-tensile strength ratio is typically above or equal to 1.1, such as 1.1-1.5. In the middle ply, the MD/CD-tensile strength ratio is typically above or equal to 1.3, such as 1.3-1.9. Typically, the MD/CD tensile strength ratio is higher for the top ply than for the back ply, and typically the MD/CD tensile strength ratio is higher for the middle ply than for the back ply. If the MD/CD tensile strength ratio is arranged in that order it has been found beneficial for crack resistance when folding. The tensile strength is measured according to ISO 1924-3:2011.

The grammage of the paperboard as well as individual plies is measured according to ISO 536:2019. The grammage of the paperboard is typically 100-450 g/m², such as 120-350 g/m², such as 125-300 g/m². The grammage of the top ply is typically 40-100 g/m². The grammage of the middle ply is typically 75-175 g/m². The grammage of the back-ply ply is typically 25-175 g/m², such as 25-75 g/m², such as 75-175 g/m². It is beneficial that the back ply has a grammage of 25-75 g/m² for a paperboard comprising at least 3 plies and that the back ply has a grammage of 75-175 g/m² for a paperboard comprising 2 plies.

The paperboard is typically coated on the top-ply. A coating may be a printing layer that facilitates printing of the board.

The second furnish typically comprises mechanical pulp, such as chemi-thermomechanical pulp (CTMP). The second furnish also typically comprises broke pulp. The second furnish also typically comprises softwood chemical pulp, such as softwood kraft pulp. The fibres of the second furnish are typically unbleached.

The fibres of the third furnish are typically unbleached.

The fibres of the first furnish are typically bleached. Since the third furnish is used to produce the top ply it is beneficial if they are bleached for printing properties. Alternatively, they are unbleached if such visual appearance is desired.

As a second aspect of the present disclosure, there is provided a method for making a two-ply paperboard, wherein the method comprises the following steps:
i. forming a top ply web from a top ply furnish comprising fibres on a top ply forming wire wherein the top ply furnish is applied on the top ply forming wire using a first jet speed at a first jet-to-wire speed difference, wherein the first jet-to-wire speed difference is in the range of:
   +12 to +30 m/min, such as +14 to +25 m/min or
   -12 to -30 m/min, such as -14 to -25 m/min
ii. forming a back ply web from a back ply furnish comprising fibres on a back ply forming wire using a second speed, wherein the second jet speed is closer to the second forming wire speed than the first jet speed to the first forming wire speed;
iii. causing the back ply web to oscillate in a direction transverse to the MD, wherein the stroke length in the oscillation of the back ply web is 10-35 mm; and
iv. combining the top ply web and back ply webs into the two-ply paperboard, wherein the top-ply web forms a top-ply and the back-ply web forms a back-ply in the two-ply paperboard.

The examples and embodiments discussed above in connection to the first aspect apply to the second aspect *mutatis mutandis.*

### EXAMPLES

### Production of a two-ply paperboard

A full-scale board machine provided with two headboxes and two wires was used. In each headbox a furnish was provided that contained fibres. The fibres for the top ply were a mixture of softwood and hardwood bleached kraft fibres and the fibres for the bottom ply were unbleached softwood kraft fibres. Trials were conducted where each furnish was applied to each wire with individual jet speeds. Both wires were running at the same speed and in Trial 1 the speed was 700 m/min. The conditions are shown in Table 1 below.

**Table 1. Jet-to-wire ratio and jet-to-wire speed difference for the top ply and bottom ply in the production of the two-ply paperboard.**

| | Trial 1 | |
|---|---|---|
| | Jet-to-wire speed difference | Jet-to-wire ratio* |
| Top ply | +16 m/min | 1.022 |
| Bottom ply | +14 m/min | 1.02 |

| | | |
|---|---|---|
| *Calculated from the wire speed and jet-to-wire speed difference | | |

The bottom plies in each trial were oscillated in a direction transverse to the machine direction (MD) by a breast roll shaker. The conditions for the breast roll shaker are shown in Table 2 below.

**Table 2. Frequency and stroke length in the oscillation with a breast roll shaker for the two-ply paperboard.**

| | Trial 1 | |
|---|---|---|
| | Frequency (rpm) | Stroke length (mm) |
| Top ply | - | - |
| Bottom ply | 400 | 25 |

### Production of a three-ply paperboard

A full-scale board machine provided with three headboxes and three wires was used. In each headbox a furnish was provided that contained fibres. The fibres for the top ply were a mixture of softwood and hardwood bleached kraft fibres. The fibres for the bottom ply were unbleached softwood kraft fibres. In the middle ply a mixture of CTMP, broke and unbleached softwood kraft fibres was used. The grammage of the top ply was about 70 g/m², the grammage of the middle ply was about 125 g/m² and the grammage of the back ply was about 50 g/m². Trials were conducted where each furnish was applied to each wire with individual jet speeds. All three wires were running at the same speed in each trial. The conditions are shown in Table 3 below.

**Table 3. Jet-to-wire ratio and jet-to-wire speed difference for the top ply, middle ply and bottom ply in the production of the three-ply paperboard.**

| Trial | | Top ply | Middle ply | Back ply |
|---|---|---|---|---|
| 2 (wire speed 669 m/min) | Jet-to-wire speed difference (m/min) | +20 | +8 | +7 |
| | Jet-to-wire ratio | 1.030 | 1.012 | 1.010 |
| 3 (wire speed 607 m/min) | Jet-to-wire speed difference (m/min) | +20 | +8 | +2 |
| | Jet-to-wire ratio | 1.030 | 1.013 | 1.003 |
| 4 (wire speed 607 m/min) | Jet-to-wire speed difference (m/min) | +20 | +20 | +5 |
| | Jet-to-wire ratio | 1.030 | 1.030 | 1.008 |

| | | | | |
|---|---|---|---|---|
| *Calculated from the wire speed and jet-to-wire speed difference | | | | |

The bottom and middle plies in each trial were oscillated in a direction transverse to the machine direction (MD) by a breast roll shaker. The conditions for the breast roll shaker are shown in Table 4 below.

**Table 4. Frequency and stroke length in the oscillation with a breast roll shaker for the three-ply paperboard.**

| Trial | | Top ply | Middle ply | Back ply |
|---|---|---|---|---|
| 2 | Stroke length (mm) | - | 25 | 14 |
| | Frequency (rpm) | - | 450 | 450 |
| 3 | Stroke length (mm) | - | 25 | - |
| | Frequency (rpm) | - | 450 | - |
| 4 | Stroke length (mm) | - | 5 | - |
| | Frequency (rpm) | - | 300 | - |

### Splitting of plies in multi-ply paperboard

Pieces of about 0.2 x 0.3 cm from a multi-ply paperboard was cut and soaked in warm water together with detergent for 20 minutes. Thereafter, the plies were separated by hand and dried individually. These plies were used for measuring of formation as they surfaces remain intact from when they were formed. It is not suitable to measure mechanical properties on plies that have been split by this wet-splitting method as the plies will shrink when drying.

Therefore, for the mechanical properties the plies were splitted by a fortuna splitter instead. Fortuna splitter is a precision bandknife splitting machine that is used to separate the plies by cutting.

### Tensile strength ratio and formation

Tensile strength was measured according to ISO 1924-3:2011.

Formation was measured according to SCAN-P 92:09.

The MD/CD tensile strength ratio, i.e. indication on how fibres are aligned in MD and CD, respectively, is presented in the tables below. Moreover, the specific formation, i.e. how homogenous in terms of local grammage variations the individual plies were, is shown.

Table 6. The MD/CD tensile strength ratio and specific formation for the two-ply paperboard.

| | Trial 1 | |
|---|---|---|
| | Top ply | Back ply |
| MD/CD-tensile strength ratio | - | 1.95 |
| Specific formation (√g/m) | - | - |

**Table 7. The MD/CD tensile strength ratio and specific formation for the three-ply paperboard.**

| Trial | | Whole board | Top ply | Middle ply | Back ply |
|---|---|---|---|---|---|
| 2 | MD/CD-tensile strength ratio | 1.8 | 2.5 | 1.5 | 1.4 |
| | Specific formation (√g/m) | 0.79 | 0.62 | 0.82 | 0.73 |
| 3 | MD/CD-tensile strength ratio | 1.7 | 2.6 | 1.5 | 1.2 |
| | Specific formation (√g/m) | 0.76 | 0.51 | 0.84 | 0.84 |
| 4 | MD/CD-tensile strength ratio | 2.1 | 2.6 | 2.4 | 1.6 |
| | Specific formation (√g/m) | 0.84 | - | 0.93 | 0.75 |

Based on the results from the crack-resistance, it is believed that an improvement, i.e. lowering, of the specific formation for the middle and back plies, is beneficial for crack resistance. Moreover, it is believed that a relatively high MD/CD tensile strength ratio for the whole board and/or in the top ply is beneficial.

Moreover, as seen in trial 2 a frequency of 150 rpm is sufficient to provide a good formation when the stroke length is 20 mm.

### Resistance to cracks and defects when folded

Different defects in the form of cracks appear when the board is folded, for example in production of a package. It is important that such cracks are as small as possible since they may otherwise cause negative effects, e.g. that the barrier is stretched too much, cracks and the content in the package is contaminated.

To evaluate the appearance of defects, packages were produced from the boards and inspection was made for various types of cracks and defects. If the cracks and defects are small, they are within acceptable limits. The results are presented in the table 5 below.

**Table 5. Visual defects detection test.**

| | Trial | | | |
|---|---|---|---|---|
| | 1 | 2 | 3 | 4 |
| Visual defects within acceptable limits when folded? | Yes | * | Yes | No |

| | | | | |
|---|---|---|---|---|
| *Not evaluated, but based on its specific formation as well as MD/CD tensile strength ratio of the individual plies and whole board, the inventors estimate that this board would be within acceptable crack limits when folded. | | | | |

Trials 1-3 representing inventive examples all pass the test, or as in the case of trial 2 is assumed to pass the test based on its properties. Trial 4 is a comparative example that failed. Based on the results, it is concluded that it is advantageous to combine a stroke length of above 10 mm for the middle ply (in case of a 3-ply board) and for the back ply (in case of a 2-ply board) with a jet-to-wire speed difference being more than +15 m/min for the top ply. Moreover, it is concluded that it is beneficial if the jet-to-wire speed difference is not being too close to o for the furnish producing the middle ply or, in case that it is also oscillated, the furnish producing the back-ply.

It is further concluded that, for a 3-layered board, a MD/CD tensile strength ratio below 2.0 is beneficial. Contributing to the MD/CD tensile strength ratio of the whole board is the MD/CD tensile strength ratio of the individual plies. It is concluded, that for a 3-layered board, it is advantageous if the MD/CD-tensile strength ratio is 1.1-1.5 for the back ply, and 1.3-1.9 for the middle ply.

It is further concluded that, for a 3-layered board, the specific formation advantageously is 0.60-0.90 √g/m for the back ply, 0.60-0.90 √g/m for the middle ply and 0.60-0.80 √g/m for the whole board.

Based on these conclusions, the inventor's estimation is that the board of trial 2 would be within acceptable crack limits when folded.

## Claims

1. A method for making a multi-ply paperboard, wherein the method comprises the following steps:
a) forming a first web from a first furnish comprising fibres on a first forming wire wherein the first furnish is applied on the first forming wire using a first jet speed at a first jet-to-wire speed difference, wherein the first jet-to-wire speed difference is in the range of:
+15 to +30 m/min, such as +16 to +25 m/min; or
-15 to -30 m/min, such as -16 to -25 m/min;
b) forming a second web from a second furnish comprising fibres on a second forming wire using a second jet speed, wherein the second jet speed is closer to the speed of the second forming wire than the first jet speed to the speed of the first forming wire;
c) forming a third web from a third furnish comprising fibres on a third forming wire using a third jet speed, wherein the third jet speed is closer to the speed of the third forming wire than the first jet speed to the speed of the first forming wire;
d) causing the second web to oscillate in a direction transverse to the machine direction (MD), wherein the stroke length in the oscillation of the second web is 10-35 mm; and
e) combining the first, second and third webs into the multi-ply paperboard, wherein the first web forms a top-ply, the second web forms a middle ply and the third web forms a back-ply in the multi-ply paperboard.

2. The method of claim 1, wherein step d) further comprises causing the third web to oscillate in a direction transverse to the machine direction.

3. The method of any one of the preceding claims, wherein the oscillation(s) in step d) is/are carried out by (a) breast roll shaker(s).

4. The method of any one of the preceding claims, wherein the stroke length in the oscillation in step d) of the second web is 12-30 mm, such as 15-30 mm.

5. The method of any one of the claims 2-4, wherein the stroke length in the oscillation in step d) of the third web is 8-25 mm, such as, 10-23 mm.

6. The method of any one of the preceding claims, wherein the wire speed of all forming wires is 400-1000 m/min, such as 500-900 m/min.

7. The method of any one of the preceding claims, wherein the second furnish comprises mechanical pulp, such as chemi-thermomechanical pulp (CTMP).

8. The method of any one of the preceding claims, wherein the second furnish comprises broke pulp.

9. The method of any one of the preceding claims, wherein the fibres of the first furnish are bleached.

10. The method of any one of the preceding claims, wherein the second furnish is applied on the second forming wire at a second jet-to-wire speed difference, which is in the range of:
+4 to +14 m/min, such as +6 to +11 m/min; or
-4 to -14 m/min, such as -6 to -11 m/min.

11. The method of any one of the preceding claims, wherein the third furnish is applied on the third forming wire at a third jet-to-wire speed difference, which is in the range of:
+4 to +14 m/min, such as +6 to +11 m/min; or
-4 to -14 m/min, such as -6 to -11 m/min.

12. The method of any one of any one of the preceding claims, wherein the third jet speed is closer to the speed of the third forming wire than the second jet speed to the speed of the second forming wire.

13. The method of any one of the preceding claims, wherein the multi-ply paperboard is coated on the top-ply.

14. The method of any one of the preceding claims, wherein the frequency in the oscillation in step d) is 130-650 rpm, such as 250-580 rpm, for the oscillated web(s).

15. A method for making a two-ply paperboard, wherein the method comprises the following steps:
i. forming a top ply web from a top ply furnish comprising fibres on a top ply forming wire wherein the top ply furnish is applied on the top ply forming wire using a first jet speed at a first jet-to-wire speed difference, wherein the first jet-to-wire speed difference is in the range of:
+12 to +30 m/min, such as +14 to +25 m/min; or
-12 to -30 m/min, such as -14 to -25 m/min;
ii. forming a back ply web from a back ply furnish comprising fibres on a back ply forming wire using a second speed, wherein the second jet speed is closer to the second forming wire speed than the first jet speed to the first forming wire speed;
iii. causing the back ply web to oscillate in a direction transverse to the MD, wherein the stroke length in the oscillation of the back ply web is 10-35 mm; and
iv. combining the top ply web and back ply webs into the two-ply paperboard, wherein the top-ply web forms a top-ply and the back-ply web forms a back-ply in the two-ply paperboard.

## Patentansprüche

1. Verfahren zum Herstellen eines mehrlagigen Kartons, wobei das Verfahren die folgenden Schritte umfasst:
a) Bilden einer ersten Bahn aus einem ersten faserhaltigen Ausgangsmaterial auf einem ersten Formiersieb, wobei das erste Ausgangsmaterial auf das erste Formiersieb unter Verwendung einer ersten Strahlgeschwindigkeit mit einer ersten Strahl-zu-Sieb-Geschwindigkeitsdifferenz aufgebracht wird, wobei die erste Strahl-zu-Sieb-Geschwindigkeitsdifferenz in folgendem Bereich liegt:
+15 bis +30 m/min, beispielsweise +16 bis +25 m/min; oder
-15 bis -30 m/min, beispielsweise -16 bis -25 m/min;
b) Bilden einer zweiten Bahn aus einem zweiten faserhaltigen Ausgangsmaterial auf einem zweiten Formiersieb unter Verwendung einer zweiten Strahlgeschwindigkeit, wobei die zweite Strahlgeschwindigkeit näher an der Geschwindigkeit des zweiten Formiersiebs liegt als die erste Strahlgeschwindigkeit an der Geschwindigkeit des ersten Formiersiebs;
c) Bilden einer dritten Bahn aus einem dritten faserhaltigen Ausgangsmaterial auf einem dritten Formiersieb unter Verwendung einer dritten Strahlgeschwindigkeit, wobei die dritte Strahlgeschwindigkeit näher an der Geschwindigkeit des dritten Formiersiebs liegt als die erste Strahlgeschwindigkeit an der Geschwindigkeit des ersten Formiersiebs;
d) Bewirken, dass die zweite Bahn in einer Richtung quer zur Maschinenrichtung (MD) oszilliert, wobei die Hublänge bei der Oszillation der zweiten Bahn 10-35 mm beträgt; und
e) Zusammenführen der ersten, der zweiten und der dritten Bahn in den mehrlagigen Karton, wobei die erste Bahn eine obere Lage bildet, die zweite Bahn eine mittlere Lage bildet und die dritte Bahn eine hintere Lage in dem mehrlagigen Karton bildet.

2. Verfahren nach Anspruch 1, wobei Schritt d) ferner Bewirken, dass die dritte Bahn in einer Richtung quer zur Maschinenrichtung oszilliert, umfasst.

3. Verfahren nach einem der vorhergehenden Ansprüche, wobei die Oszillation(en) in Schritt d) durch (einen) Brustwalzenschüttler ausgeführt wird/werden.

4. Verfahren nach einem der vorhergehenden Ansprüche, wobei die Hublänge bei der Oszillation in Schritt d) der zweiten Bahn 12-30 mm, beispielsweise 15-30 mm, beträgt.

5. Verfahren nach einem der Ansprüche 2-4, wobei die Hublänge bei der Oszillation in Schritt d) der dritten Bahn 8-25 mm, beispielsweise 10-23 mm, beträgt.

6. Verfahren nach einem der vorhergehenden Ansprüche, wobei die Siebgeschwindigkeit aller Formiersiebe 400-1000 m/min, beispielsweise 500-900 m/min, beträgt.

7. Verfahren nach einem der vorhergehenden Ansprüche, wobei das zweite Ausgangsmaterial mechanischen Holzstoff, beispielsweise chemo-thermomechanischen Holzstoff (CTMP), umfasst.

8. Verfahren nach einem der vorhergehenden Ansprüche, wobei das zweite Ausgangsmaterial Halbstoffausschuss umfasst.

9. Verfahren nach einem der vorhergehenden Ansprüche, wobei die Fasern des ersten Ausgangsmaterials gebleicht sind.

10. Verfahren nach einem der vorhergehenden Ansprüche, wobei das zweite Ausgangsmaterial auf das zweite Formiersieb mit einer zweiten Strahl-zu-Sieb-Geschwindigkeitsdifferenz aufgebracht wird, die in folgendem Bereich liegt:
+4 bis +14 m/min, beispielsweise +6 bis +11 m/min; oder
-4 bis -14 m/min, beispielsweise -6 bis -11 m/min.

11. Verfahren nach einem der vorhergehenden Ansprüche, wobei das dritte Ausgangsmaterial auf das dritte Formiersieb mit einer dritten Strahl-zu-Sieb-Geschwindigkeitsdifferenz aufgebracht wird, die in folgendem Bereich liegt:
+4 bis +14 m/min, beispielsweise +6 bis +11 m/min; oder
-4 bis -14 m/min, beispielsweise -6 bis -11 m/min.

12. Verfahren nach einem der vorhergehenden Ansprüche, wobei die dritte Strahlgeschwindigkeit näher an der Geschwindigkeit des dritten Formiersiebs liegt als die zweite Strahlgeschwindigkeit an der Geschwindigkeit des zweiten Formiersiebs.

13. Verfahren nach einem der vorhergehenden Ansprüche, wobei der mehrlagige Karton auf der oberen Lage beschichtet wird.

14. Verfahren nach einem der vorhergehenden Ansprüche, wobei die Frequenz bei der Oszillation in Schritt d) 130-650 U/min, beispielsweise 250-580 U/min, für die oszillierte(n) Bahn(en) beträgt.

15. Verfahren zum Herstellen eines zweilagigen Kartons, wobei das Verfahren die folgenden Schritte umfasst:
i. Bilden einer Bahn einer oberen Lage aus einem faserhaltigen Ausgangsmaterial für eine obere Lage auf einem Formiersieb für eine obere Lage, wobei das Ausgangsmaterial für die obere Lage auf das Formiersieb für die obere Lage unter Verwendung einer ersten Strahlgeschwindigkeit mit einer ersten Strahl-zu-Sieb-Geschwindigkeitsdifferenz aufgebracht wird, wobei die erste Strahl-zu-Sieb-Geschwindigkeitsdifferenz in folgendem Bereich liegt:
+12 bis +30 m/min, beispielsweise +14 bis +25 m/min; oder
-12 bis -30 m/min, beispielsweise -14 bis -25 m/min;
ii. Bilden einer Bahn einer hinteren Lage aus einem faserhaltigen Ausgangsmaterial für eine hintere Lage auf einem Formiersieb für eine hintere Lage unter Verwendung einer zweiten Geschwindigkeit, wobei die zweite Strahlgeschwindigkeit näher an der zweiten Formiersiebgeschwindigkeit liegt als die erste Strahlgeschwindigkeit an der ersten Formiersiebgeschwindigkeit;
iii. Bewirken, dass die Bahn der hinteren Lage in einer Richtung quer zur MD oszilliert, wobei die Hublänge bei der Oszillation der Bahn der hinteren Lage 10-35 mm beträgt; und
iv. Zusammenführen der Bahn der oberen Lage und der Bahnen der hinteren Lage in den zweilagigen Karton, wobei die Bahn der oberen Lage eine obere Lage bildet und die Bahn der hinteren Lage eine hintere Lage in dem zweilagigen Karton bildet.

## Revendications

1. Procédé de production d'un carton multicouche, dans lequel le procédé comprend les étapes suivantes :
a) former une première feuille continue à partir d'une première composition de fabrication, comprenant des fibres, sur une première toile de formation, dans lequel la première composition de fabrication est appliquée sur la première toile de formation en utilisant une première vitesse de jet à une première différence de vitesse jet-toile, dans lequel la première différence de vitesse jet-toile est dans la plage de :
+15 à +30 m/min, telle que de +16 à +25 m/min ; ou
-15 à -30 m/min, telle que de -16 à -25 m/min ;
b) former une deuxième feuille continue à partir d'une deuxième composition de fabrication, comprenant des fibres, sur une deuxième toile de formation en utilisant une deuxième vitesse de jet, dans lequel la deuxième vitesse de jet est plus proche de la vitesse de la deuxième toile de formation que la première vitesse de jet n'est de la vitesse de la première toile de formation ;
c) former une troisième feuille continue à partir d'une troisième composition de fabrication, comprenant des fibres, sur une troisième toile de formation en utilisant une troisième vitesse de jet, dans lequel la troisième vitesse de jet est plus proche de la vitesse de la troisième toile de formation que la première vitesse de jet n'est de la vitesse de la première toile de formation ;
d) amener la deuxième feuille continue à osciller dans un sens transversal au sens machine (MD), dans lequel la longueur de course dans l'oscillation de la deuxième feuille continue est de 10 à 35 mm ; et
e) combiner les première, deuxième, et troisième feuilles continues en le carton multicouche, dans lequel la première feuille continue forme une couche supérieure, la deuxième feuille continue forme une couche intermédiaire, et la troisième feuille continue forme une couche arrière dans le carton multicouche.

2. Procédé de la revendication 1, dans lequel l'étape d) comprend en outre amener la troisième feuille continue à osciller dans un sens transversal au sens machine.

3. Procédé de l'une quelconque des revendications précédentes, dans lequel la ou les oscillation(s) dans l'étape d) est/sont effectuée(s) par (a) un ou des vibreur(s) de rouleau de tête.

4. Procédé de l'une quelconque des revendications précédentes, dans lequel la longueur de course dans l'oscillation dans l'étape d) de la deuxième feuille continue est de 12 à 30 mm, telle que de 15 à 30 mm.

5. Procédé de l'une quelconque des revendications 2 à 4, dans lequel la longueur de course dans l'oscillation dans l'étape d) de la troisième feuille continue est de 8 à 25 mm, telle que de 10 à 23 mm.

6. Procédé de l'une quelconque des revendications précédentes, dans lequel la vitesse de toile de toutes les toiles de formation est de 400 à 1000 m/min, telle que de de 500 à 900 m/min.

7. Procédé de l'une quelconque des revendications précédentes, dans lequel la deuxième composition de fabrication comprend de la pâte mécanique, telle que de de la pâte chimio-thermomécanique (« Chemi-TermoMechanical Pulp », CTMP).

8. Procédé de l'une quelconque des revendications précédentes, dans lequel la deuxième composition de fabrication comprend de la pâte de cassés.

9. Procédé de l'une quelconque des revendications précédentes, dans lequel les fibres de la première composition de fabrication sont blanchies.

10. Procédé de l'une quelconque des revendications précédentes, dans lequel la deuxième composition de fabrication est appliquée sur la deuxième toile de formation à une deuxième différence de vitesse jet-toile, qui est dans la plage de :
+4 à +14 m/min, telle que de +6 à +11 m/min ; ou
-4 à -14 m/min, telle que de -6 à -11 m/min.

11. Procédé de l'une quelconque des revendications précédentes, dans lequel la troisième composition de fabrication est appliquée sur la troisième toile de formation à une troisième différence de vitesse jet-toile, qui est dans la plage de :
+4 à +14 m/min, telle que de +6 à +11 m/min ; ou
-4 à -14 m/min, telle que de -6 à -11 m/min.

12. Procédé de l'une quelconque des revendications précédentes, dans lequel la troisième vitesse de jet est plus proche de la vitesse de la troisième toile de formation que la deuxième vitesse de jet n'est de la vitesse de la deuxième toile de formation.

13. Procédé de l'une quelconque des revendications précédentes, dans lequel le carton multicouche est revêtu sur la couche supérieure.

14. Procédé de l'une quelconque des revendications précédentes, dans lequel la fréquence dans l'oscillation dans l'étape d) est de 130 à 650 tr/min, telle que de 250 à 580 tr/min, pour la ou les feuille(s) continue(s) amenée(s) en oscillation.

15. Procédé de production d'un carton à deux couches, dans lequel le procédé comprend les étapes suivantes :
i. former une feuille continue de couche supérieure à partir d'une composition de fabrication de couche supérieure, comprenant des fibres, sur une toile de formation de couche supérieure, dans lequel la composition de fabrication de couche supérieure est appliquée sur la toile de formation de couche supérieure en utilisant une première vitesse de jet à une première différence de vitesse jet-toile, dans lequel la première différence de vitesse jet-toile est dans la plage de :
+12 à +30 m/min, telle que de +14 à +25 m/min ; ou
-12 à -30 m/min, telle que de -14 à -25 m/min ;
ii. former une feuille continue de couche arrière à partir d'une composition de fabrication de couche arrière, comprenant des fibres, sur une toile de formation de couche arrière en utilisant une deuxième vitesse, dans lequel la deuxième vitesse de jet est plus proche de la deuxième vitesse de toile de formation que la première vitesse de jet n'est de la première vitesse de toile de formation ;
iii. amener la feuille continue de couche arrière à osciller dans un sens transversal au MD, dans lequel la longueur de course dans l'oscillation de la feuille continue de couche arrière est de 10 à 35 mm ; et
iv. combiner la feuille continue de couche supérieure et la feuille continue de couche arrière en le carton à deux couches, dans lequel la couche supérieure feuille continue forme une couche supérieure et la couche arrière feuille continue forme une couche arrière dans le carton à deux couches.
